

C. F. GRABER,  
PYROTECHNIC DEVICE.  
APPLICATION FILED OCT. 5, 1907.

902,650.

Patented Nov. 3, 1908.



WITNESSES:

*F. H. W. Fraenzel*  
*Anna H. Deter*

INVENTOR:

*Charles F. Graber*  
BY  
*Fraenzel and Richards*,  
ATTORNEYS

# UNITED STATES PATENT OFFICE.

CHARLES F. GRABER, OF DALLAS, TEXAS, ASSIGNOR TO EDWARD H. WAGNER, OF NEW YORK, N. Y.

## PYROTECHNIC DEVICE.

No. 902,650.

Specification of Letters Patent.

Patented Nov. 3, 1908.

Application filed October 5, 1907. Serial No. 395,993.

*To all whom it may concern:*

Be it known that I, CHARLES F. GRABER, a citizen of the United States, residing at Dallas, in the county of Dallas and State of Texas, have invented certain new and useful Improvements in Pyrotechnic Devices; and I do hereby declare the following to be a full, clear, and exact description of the invention, such as will enable others skilled in the art to 10 which it appertains to make and use the same, reference being had to the accompanying drawings, and to characters of reference marked thereon, which form a part of this specification.

15 This invention relates, generally, to improvements in pyrotechnic devices; and, the invention relates, more particularly, to a pyrotechnic device comprising a suitable pyrotechnic composition capable of being 20 exploded by percussion and inclosed with a safety-coating, so as to provide a device of the general character hereinafter more fully set forth which shall be free from accidental ignition due to any friction caused in handling the device, or while carrying the same 25 in the pocket, or while in transmission when packed for shipment from place to place.

My present invention has for its principal object to provide a new and simple, as well as 30 a perfectly safe pyrotechnic device known in the art as crazy crackers; and, the invention has for its further object to provide a novel pyrotechnic device which shall be perfectly safe against accidental ignition due to friction in the handling or shipping of the finished product.

Other objects of this invention not at this time more particularly enumerated will be clearly evident from the following detailed 40 description.

My invention consists, primarily, in the novel pyrotechnic device hereinafter more fully described, and in the novel process or method of making the same.

45 In the accompanying drawing is illustrated in transverse section, on an enlarged scale, a crazy cracker showing one of the uses to which my novel pyrotechnical compound may be put, the crazy cracker being ignited 50 by scratching, as in the manner of igniting a match, or by throwing the article down upon a hard surface, in the manner of the usual hand-torpedoes.

In the said drawing, the reference-character 55 1 indicates the pyrotechnic device, 2 rep-

resents a shell or covering of thin tissue paper, or other suitable tissue or material, 3 is a suitable covering glue, dextrin, or other suitable surface of a gummy or sticky nature, and 4 is a protective shell or coating, as 60 wood-pulp or the like, which serves as a safety covering or protection against the accidental ignition of the pyrotechnic device while the same is being handled, or while packed in boxes and cases and in transit 65 from place to place.

The pyrotechnical composition of matter usually employed for the pyrotechnic device is manufactured in the following manner.

Ten pounds of thick gum-arabic with sufficient water, say about one gallon are placed in a vessel and heated to provide a comparatively thin but sticky mass. To this mass is then added one pound and fourteen ounces of stick or white phosphorus, the latter becoming 70 intimately intermingled or mixed with the gum-arabic and water in said sticky mass while the latter is agitated and while it is kept hot. As soon as the several ingredients have been thoroughly incorporated, 75 three pounds and six ounces of carbonate of magnesium are added. The mixture is then allowed to cool, while still stirring or agitating the mass, so as to obtain an intimate mixture. Six pounds of chlorate of potash 80 rapidly stirred in one pint of boiling water so as to produce a paste-like mass, are then added so as to obtain a plastic or putty-like mass. Pieces of thin tissue are then placed in suitable molds and the plastic or putty- 85 like mass poured or put upon each piece of paper in the depression of a mold. After folding over the projecting edge-portion of the tissue paper or other thin material used 90 the article or body thus formed is tamped 95 tight and removed from the mold and allowed to dry. The bodies are then dipped into liquid glue, gum, dextrin, or other suitable liquid of a gum-like or sticky nature, so as to produce the hereinabove mentioned 100 surface 3, which is then finally coated with a protective material, such as wood pulp or a material of a similar nature, the same being sifted upon or otherwise applied to the still gummy or sticky surface 3, so as to adhere to 105 the same and thereby produce the shell or coating 4 previously mentioned, which as soon as the finished product has finally dried forms a suitable safety covering against the accidental ignition of the pyrotechnical com- 110

pound by friction caused by the rubbing together of two or more of the finished articles.

From the foregoing description of my present invention it will be clearly evident 5 that I have produced a pyrotechnic device which is perfectly safe from premature or accidental ignition.

The composition usually consists of the above-mentioned ingredients, preferably by 10 the weights stated, but it will be understood, and I am fully aware of the fact that the proportions of the ingredients by weight may be changed without departing from the spirit and scope of the present invention, as set 15 forth in the appended claims. Hence I do not limit my invention to the exact proportions of the various ingredients named in the foregoing specification.

I claim:—

20 1. The herein described pyrotechnic device comprising a suitable pyrotechnic composition capable of being exploded by per-

cussion and inclosed within a safety-coating comprising a wrapper of tissue paper having its outer surface gummed, and a protecting 25 coating adhering to said gummed surface, substantially as described.

2. The herein described pyrotechnic device comprising a suitable pyrotechnic composition capable of being exploded by percussion and inclosed within a safety-coating comprising a wrapper of tissue paper having its outer surface gummed, and a layer of wood-pulp adhering to said gummed surface, substantially as and for the purposes set 30 35 forth.

In testimony, that I claim the invention set forth above I have hereunto set my hand this thirtieth day of September, 1907.

CHARLES F. GRABER.

Witnesses:

GEORGE D. RICHARDS,  
EVELYN R. LESSER.